

United States Patent [19]  
Procter

[11] 3,929,559  
[45] Dec. 30, 1975

[54] STABILIZATION OF CELLULOSIC MATERIAL BY TREATMENT WITH FERRICYANIDE ION

3,663,358 5/1972 Falkenhag et al. .... 162/70  
3,883,391 5/1975 Phillips ..... 162/70 X

[75] Inventor: Alan R. Procter, North Vancouver, Canada

Primary Examiner—S. Leon Bashore  
Assistant Examiner—Arthur L. Corbin  
Attorney, Agent, or Firm—Larson, Taylor and Hinds

[73] Assignee: MacMillan Bloedel Limited, Vancouver, Canada

[22] Filed: Dec. 16, 1974

[57] ABSTRACT

[21] Appl. No.: 533,027

A method of stabilizing a cellulosic material against degradation by an aqueous alkaline medium. The cellulosic material is treated with a ferricyanide ion under alkaline conditions. The preferred application of the method is in the production of pulp for paper making and the preferred cellulosic material is thus wood. The treating with the ferricyanide ion may take place prior to the pulping or during the pulping.

[52] U.S. Cl. .... 162/70; 8/116 R; 162/90  
[51] Int. Cl.<sup>2</sup> .... D21C 1/00; D21C 1/06  
[58] Field of Search ..... 162/70, 90; 8/116 R

[56] References Cited

UNITED STATES PATENTS

3,532,596 10/1970 Bills et al. .... 162/70

13 Claims, 1 Drawing Figure

RELATION BETWEEN PULP YIELD AND KAPPA NUMBER  
FOR SODA COOKS OF WESTERN HEMLOCK CHIPS



◎=SODA PULP USING FERRICYANIDE STABILIZATION

## STABILIZATION OF CELLULOSIC MATERIAL BY TREATMENT WITH FERRICYANIDE ION

### BACKGROUND OF THE INVENTION

#### 1. FIELD OF THE INVENTION

This invention relates to a stabilization of carbohydrate material against degradation by an aqueous alkaline medium.

#### 2. DESCRIPTION OF THE PRIOR ART

Paper may be defined as a tissue of fibrous cellulosic materials. The individual cellulose fibres of the original raw material from which the paper is made are first separated from one another by chemical or mechanical means and then felted together to form the tissue. The principal source of cellulosic material used in paper making is wood. It is desirable that the cellulose used in paper making should be as pure as possible but in wood the cellulose fibres are intimately associated with incrustants, principally lignin. To isolate the cellulose from the incrustants the wood is pulped as the first step in the main paper making process.

The pulping of wood to make wood pulp may be divided into four main groups:

- i. Mechanical or ground wood pulp is prepared by a mechanical disintegration of the wood in the presence of water. Yields may be approximately 95%.
- ii. Chemi-mechanical pulp is obtained by softening the wood by a very mild chemical treatment without significant delignification and then disintegrating the wood by mechanical action. Typically sodium hydroxide, for example at 30° to 80°C, is used. Yields are typically in the range of 80 to 95%.
- iii. Semi-chemical pulp is obtained by stronger chemical action than in chemi-mechanical pulping. Conditions are such that some delignification occurs. The chemical action is followed by defibering by mechanical treatment. Typical yields are 55 to 80%. The reagent originally used in semi-chemical pulping was neutral sodium sulfite, that is sodium sulfite buffered by sodium carbonate. But later it was realized that the reagents useful in the full chemical pulping of wood were useful if milder reaction conditions were employed and if it were ensured that the digestion or pulping process was stopped before any major delignification occurred. Thus acid sulfite (calcium bisulfite and sulfuric acid); bisulfite (a mixture of sodium bisulfite and magnesium bisulfite) and sulfate (sodium hydroxide and sodium sulfide) are now used in semi-chemical pulping.
- iv. Chemical pulp is obtained by chemical treatment sufficient to remove the interfibre lignin of the wood thus allowing the cellulose fibres to separate with only minor or no mechanical treatment. A typical yield is 42 to 58% depending on the wood used and the digestion chemical.

Chemical pulping has been subdivided to alkaline pulping and acid pulping. Alkaline pulping may be further subdivided into the soda process in which sodium hydroxide is used to carry out the pulping process and the kraft or sulfate process in which sodium hydroxide and sodium sulfide are used.

The present invention finds applications in the alkaline pulping of carbohydrate material, particularly wood.

The original alkaline pulping process was the use of sodium hydroxide. Because of the cost of sodium hydroxide it was necessary to recover the sodium hydrox-

ide in the residual or black liquor and to re-use it. This recovery was by separation and evaporation of the black liquor, burning and dissolving the resultant sodium carbonate in water. Calcium hydroxide was then added to the solution to obtain sodium hydroxide. It was later found that sodium sulfide in the cooking liquor gave improved dissolution and less degraded pulp. By using sodium sulfate to make up the sodium hydroxide loss and adding it to the black liquor before burning

the makeup sulfate was reduced to the desired sodium sulfide. The use of sodium sulfate rather than sodium hydroxide for makeup gives the name the sulfate process. However, the process is principally known as the kraft process.

All the chemical pulping processes suffer from the disadvantage that cellulose can undergo many chemical transformations. Thus the pulping process, in delignifying wood, also destroys cellulose and the associated hemicelluloses. Although the kraft process is the most widely used alkaline pulping process because of its well-established technology and ability to produce strong pulps from practically any fibrous lignocellulosic material it has the disadvantages, first, of low yield and, secondly, that it produces an unpleasant odour associated with sulfur-containing gaseous emission. For the past several years it has been a major concern of the pulping industry to find a sulfur-free pulping process in which these emissions would be avoided. One process suggested for the avoiding of the emissions is the soda process mentioned above. However this process suffers from the disadvantage that even lower pulp yield is achieved than with the kraft process, again as a result of carbohydrate alkaline degradation.

U.S. Pat. No. 3,532,596 to Bills et al discloses a process for pulping lignocellulosic material which involves treatment with an aqueous solution containing cyanide ions. By this means the aldehyde groups in the carbohydrates are converted to cyanohydrin groups and these groups then hydrolyzed into carboxyl groups. Thus the process essentially involves the incorporation of additional carbon atoms into the chain. The pulping described in U.S. Pat. No. 3,532,596 is an alkaline pulping.

U.S. Pat. No. 3,663,358 to Falkenhag et al also discloses the use of the cyanide ion to increase the pulp yield from lignocellulosic material. In this patent the pulping is carried out with a bisulfite pulping solution having a pH below 7.

The processes of the above patents proceed by a mechanism similar to the Kiliani-Fischer reaction. The mechanism is:



An obvious disadvantage of the processes described in the above patents is the extreme toxicity of the cyanide ion.

### SUMMARY OF THE INVENTION

The present invention seeks to avoid the above disadvantages by providing a method for stabilizing a carbohydrate material against degradation by an aqueous alkaline medium that comprises treating the carbohydrate material with ferricyanide ion under alkaline

conditions. The treatment with the ferricyanide ion may be carried out prior to an alkaline pulping process or during that process. The method has the virtue that the stabilized carbohydrate material is more resistant towards degradation by alkali. It is possible to pulp the stabilized carbohydrate material simply by an alkali, without sulfur compounds. Thus the method of the invention permits a sulfur-free pulping method that gives higher yields than presently possible without the disadvantage of foul smelling emissions.

In contrast to the mechanism of the above Bills et al and Falkenhag patents the mechanism of the present process is:



That is the alkaline ferricyanide acts as an oxidizing agent and is reduced to ferrocyanide. Ferricyanide is a stable ion and does not dissociate significantly into cyanide ions, a considerable advantage from the point of view of toxicity. Furthermore, the ferrocyanide ion is relatively easy to convert back to the ferricyanide ion, for example, by oxidation with air, oxygen or chlorine. This can be economically attractive.

#### DESCRIPTION OF THE PREFERRED EMBODIMENTS

In the preferred embodiments the carbohydrate material is a lignocellulosic material, for example wood. The treatment with the ferricyanide ion is generally carried out at a pH of about 10. The ferricyanide ion may be added as sodium ferricyanide or potassium ferricyanide. Although the invention has the virtue that it permits the use of the soda process and obtains good yields without foul emissions it is also possible to improve the yield of the kraft process because of the improved stability of the carbohydrate material.

The invention is illustrated in the following examples and in the attached drawing, referred to in Example 3.

#### EXAMPLE 1

Solutions of potassium ferricyanide in the presence of a  $\text{Na}_2\text{CO}_3 - \text{NaHCO}_3$  buffer system at a pH of 10 were used to pretreat hydrocellulose samples for 120 minutes at 100°C. The treated hydrocellulose samples were then washed free of spent pretreatment solution and degraded with 1N NaOH under standard conditions (100°C., 2 hours).

| Results:                                 |                                                       |
|------------------------------------------|-------------------------------------------------------|
| Molarity of Ferricyanide in Pretreatment | % Hydrocellulose Remaining After Alkaline Degradation |
| 0                                        | 29                                                    |
| 0.01 M                                   | 51                                                    |
| 0.02 M                                   | 66                                                    |
| 0.05 M                                   | 66                                                    |
| 0.2 M                                    | 72                                                    |

These results demonstrate the effectiveness of the method, when used as a pretreatment, for stabilizing cellulose towards alkaline degradation.

#### EXAMPLE 2

In the second series of experiments, potassium ferricyanide was added to alkaline digestions of hydrocellulose (100°C., 2 hours).

| Results:                       |                                                       |
|--------------------------------|-------------------------------------------------------|
| Molarity of Ferricyanide Added | % Hydrocellulose Remaining After Alkaline Degradation |
| 0                              | 29                                                    |
| 0.02 M                         | 86                                                    |
| 0.05 M                         | 86                                                    |
| 0.2 M                          | 85                                                    |

The results demonstrate the effectiveness of ferricyanide as an addition reagent to an alkaline digestion, for stabilizing cellulose toward alkaline degradation.

#### EXAMPLE 3

Potassium ferricyanide was also evaluated as a pretreatment and addition reagent in the soda pulping of western hemlock wood chips. Pretreatments were carried out by treating wood chips with an alkaline (pH 10) solution of ferricyanide at 100°C. for 2 hours. The soda pulping was carried out in small pressure bombs containing 10 g of wood chips and 200 g of 1N-Sodium Hydroxide. Cooking conditions were normally 1 hour at 170°C.

| Ferricyanide Addition | Pulp Yield | Kappa No. | Yield Increase Over An Equivalent Soda Pulp At The Same Kappa No. |
|-----------------------|------------|-----------|-------------------------------------------------------------------|
| 0.01 M                | 50.4       | 102       | + 1%                                                              |
| 0.02 M                | 51.1       | 96        | + 2                                                               |
| 0.05 M                | 55.6       | 95        | + 7                                                               |
| 0.02 M                | 51.5       | 82        | + 5                                                               |
| 0.02 M                | 55.5       | 99        | + 6                                                               |
| 0.02 M                | 63.2       | 111       | +12                                                               |

The Kappa No. is the number of milliliters of 0.1N potassium permanganate consumed by one gram of dry cellulose pulp under specified conditions. It is useful as an index related to the degree of delignification attained during the cook.

These results demonstrate the effectiveness of a ferricyanide treatment for increasing pulp yield, when compared with the yield vs. Kappa No. relationship for regular soda pulps of the same raw material. The results are illustrated graphically in FIG. 1 which compares pulp yield and Kappa No. for soda cooks of western hemlock chips with and without the ferricyanide.

The stabilizing method appears particularly effective as a pretreatment for producing high yield, high Kappa number pulps. These pulps would be particularly suitable for subsequent delignification with oxygen under pressure to produce high yield bleachable grade chemical pulps, by methods well known in the art of pulping.

It should be emphasized that the invention is useful in any process for isolating cellulose from a natural source of cellulose, for example, wood from deciduous and coniferous trees, reeds, bamboo and cotton fibres.

What I claim as my invention is:

1. A method for stabilizing a cellulosic material against degradation by an aqueous alkaline medium that comprises treating the cellulosic material with ferricyanide ion under alkaline conditions.
2. A method as claimed in claim 1 in which the treatment with the ferricyanide ion is carried out prior to contacting the cellulosic material with the aqueous alkaline medium.

3. A method as claimed in claim 1 in which the treatment with the ferricyanide ion is carried out during contact with the aqueous alkaline medium.

4. A method as claimed in claim 1 in which the cellulosic material is a lignocellulosic material.

5. A method as claimed in claim 4 in which the lignocellulosic material is wood.

6. A method as claimed in claim 1 in which the cellulosic material is cellulose.

7. A method as claimed in claim 1 in which treatment with the ferricyanide ion is carried out at a pH of about 10.

8. A method as claimed in claim 1 in which the ferricyanide ion is added as potassium ferricyanide.

9. A method as claimed in claim 1 in which the ferricyanide ion is added as sodium ferricyanide.

10. In a process for the production of pulp useful in paper-making by the alkaline pulping of a lignocellulosic material the improvement comprising treating the lignocellulosic material with an alkaline solution of ferricyanide prior to the pulping.

11. A process as claimed in claim 10 in which the alkaline pulping is by the soda process.

12. In a process for the production of pulp useful in paper-making by the alkaline pulping of a lignocellulosic material the improvement comprising treating the lignocellulosic material with the ferricyanide ion during the alkaline pulping.

13. A process as claimed in claim 12 in which the alkaline pulping is by the soda process.

\* \* \* \* \*

20

25

30

35

40

45

50

55

60

65